

## UNITED STATES PATENT OFFICE

HENRY DREYFUS, OF LONDON, ENGLAND

## TREATMENT OF CELLULOSE PREPARATORY TO ESTERIFICATION

No Drawing. Original application filed April 18, 1923, Serial No. 633,016, and in Great Britain May 24, 1922. Divided and this application filed March 15, 1929. Serial No. 347,456.

This application is a division of my prior application Serial No. 633,016 filed April 18, 1923.

The above application covers esterifying cellulose or its near conversion products with acetic or other fatty acid anhydride in presence of sulphuric acid or other strong condensing agent to produce a highly viscous product by means of using acetic acid or other solvent in quantity over six times the weight of the cellulose.

The subject-matter of the present application relates to a preliminary treatment which may be given the cellulose or cellulose conversion products in order to render them more reactive to the esterification process while substantially preserving the strength of the cellulosic material. While cellulose or its conversion products which have been pre-treated according to the process hereinafter described and claimed are especially suitable for esterification according to the process disclosed and claimed in said parent application, nevertheless they may be esterified by other known or new processes of esterification.

While the pretreatment as hereinafter described is carried out by the use of acetic acid, nevertheless, it may be carried out by the use of other fatty acids, such as propionic, butyric, or formic acid.

In carrying out the invention, the cellulose or conversion product may be first treated with acetic acid alone, either with heating or at ordinary temperature or with cooling, and sulphuric acid or other strong condensing agent, preferably diluted in acetic acid, be then added at ordinary temperature or with cooling or strong cooling, and the acetic anhydride be then introduced to effect the esterification; or the cellulose or conversion product may be first treated with acetic acid alone, either with heating or at ordinary temperature or with cooling, and then the acetic anhydride be added, the sulphuric acid or strong condensing agent being only added afterwards to the preferably cooled mass; or the cellulose or conversion product may be treated with a mixture of acetic acid and sulphuric acid or other strong condensing agent while preferably cooling or strongly

cooling, and the esterification be then effected with the acetic anhydride; or the cellulose or conversion product may be introduced into the mixture of acetic acid, acetic anhydride and sulphuric acid or condensing agent. Or the sulphuric acid or condensing agent, preferably diluted in acetic acid or acetic anhydride, may be introduced into the mixture of acetic acid, acetic anhydride and cellulose. Or the order or manner in which the respective materials are brought together or incorporated may be varied in any other suitable or desired way. With sulphuric acid or like strong condensing agents, cooling to low temperatures of for example below 5° C. and preferably 0° C. or lower should be employed at the beginning of the esterification or when the cellulose or conversion product comes in contact with esterifying agent and sulphuric acid or strong condensing agent, precooling being preferably employed with this object.

Further, I may employ for esterification according to the present invention, whether in solution or suspension, cellulose or cellulose conversion products which have been subjected to pre-treatment of the character hereinafter mentioned, to render them more reactive while substantially preserving the strength of the cellulosic material.

According to such special pretreatment the cellulose or cellulose conversion product may be heated or boiled with concentrated or dilute acetic acid or other organic acids, preferably with the addition of small quantities of sodium acetate or other and suitable neutralizing agents capable of neutralizing any traces of mineral acids that may be present, and which could have a destructive effect on the cellulose molecule in the hot treatment with organic acid. For example the cellulosic material may be heated with glacial or dilute acetic acid, preferably containing a small quantity of sodium acetate or other suitable neutralizing agent, at temperatures and for times which may vary with the concentration of the acid used, the time of treatment increasing with decreasing concentration of acid and with reduction of temperature. For instance with glacial acetic

acid at about 100° C. or at boiling temperature of the acid, the treatment may last about 1 to 6 hours more or less. The pretreatment with acetic or other organic acids may also take place in the cold, though this may prolong the time of treatment.

In any of the forms of pretreatment above referred to the acetic or other organic acid used for the pretreatment may be employed 10 in admixture with diluents not capable of entering into reaction with the cellulose or acid, such as toluol, but with less advantage.

The pretreated material may be used direct for subjection to the esterifying reaction, but 15 preferably it is washed and dried before it is esterified.

When cellulose or conversion products pre-treated as referred to are used for the esterification, this goes much more quickly, so that 20 it is even possible to conduct and finish an acetylation at temperatures as low as or lower than 0° C., though of course, especially as the esterification reaction with such pretreated materials goes much more quickly, high temperatures 25 may be used by using increased quantities of acetic acid or diluent in accordance with the present invention.

#### Example 1

30 100 parts by weight of cellulose, for example cotton, are introduced into a mixture of 800 parts by weight of glacial acetic acid, 15%-20% of sulphuric acid relatively to the weight of the cellulose, and about 200 to 250 parts by weight of acetic anhydride, this mixture having been first cooled down to 0° C.; the temperature is allowed to rise gradually, cooling being continued until complete solution. The reaction is complete in about 2 40 to 6 hours. If desired, the temperature towards the end of the reaction may be allowed to rise to 25° or 30° C. or even somewhat more to finish the reaction. The cellulose acetate obtained is of much higher viscosity than any hitherto known, as is proved by the fact that the acetylation solution obtained is, in spite of the 70% greater dilution, just as viscous as the best acetylation solutions previously obtainable. The product 45 can be isolated and employed as such or be submitted to a secondary or further treatment either in the original acetylation solution or after isolation therefrom. The isolation of the product from the acetylation solution 50 may be effected by precipitating it in water or with water or with diluents such as carbon tetrachloride and so forth.

#### Example 2

60 100 parts by weight of cellulose, for example cotton, are treated with 900 to 1,000 parts by weight of glacial acetic acid and 10 to 15 parts by weight of sulphuric acid for about 1 to 2 hours. Into the mixture, cooled to 65 about 0°-10° C. or still lower, are introduced

200 parts of acetic anhydride, the mass being constantly mixed or worked while maintaining cooling until complete solution, so that the temperature is only allowed to rise gradually to about 10° to 15° C. If desired, the 70 temperature may be allowed to rise to 20°-25° C. to complete the reaction or even to about 30° C. The acetylation reaction is finished in about 1 to 3 hours.

Instead of introducing the sulphuric acid 75 with the acetic acid in the preliminary treatment, it may be introduced after treatment with acetic acid, with or without cooling, but preferably with cooling.

Although of particular value in the production of cellulose acetate the pretreatment which forms the subject-matter of the present invention is of value in the production of any of the fatty acid esters of cellulose. The invention is, therefore, to be regarded as 85 limited only by the scope of the appended claims.

What I claim and desire to secure by Letters Patent is:—

1. A process of preparing cellulose for 90 acetylation which consists in mixing the cellulose with acetic acid of such strength that the acid crystallizes when cooled and then cooling the mixture until crystallization of the acid has occurred throughout the mass. 95

2. A process of preparing cellulose for esterification which consists in mixing the cellulose with acetic acid of such strength that the acid crystallizes when cooled and then cooling the mixture until crystallization of 100 the acid has occurred throughout the mass.

3. A process of preparing cellulose for esterification which consists in mixing the cellulose with glacial acetic acid and then cooling the mixture to a temperature below 10° C. 105

4. A process of preparing cellulose for esterification which consists in mixing the cellulose with glacial acetic acid and then cooling the mixture to a temperature below 0° C.

5. A process of preparing cellulose for esterification which consists in mixing the cellulose with a mixture of glacial acetic acid and sulphuric acid and then cooling the mixture until crystallization of the acetic acid has occurred throughout the mass. 110

In testimony whereof I have hereunto subscribed my name.

HENRY DREYFUS.

120

125

130